

Oct. 24, 1944.

E. R. WHITE ET AL

2,361,339

METAL DEACTIVATORS

Filed June 8, 1940

Oxygen absorbed  
ml. per 100 grams of oil



Inventors: Ellis R. White  
Ernest L. Walters

By their Attorney: D. Flusin

Patented Oct. 24, 1944

2,361,339

# UNITED STATES PATENT OFFICE

2,361,339

## METAL DEACTIVATORS

Ellis R. White, Albany, and Ernest L. Walters,  
San Francisco, Calif., assignors to Shell De-  
velopment Company, San Francisco, Calif., a  
corporation of Delaware

Application June 8, 1940, Serial No. 339,508

8 Claims. (Cl. 252—51)

This invention relates to a method for the stabilization of organic substances and particularly to the protection of organic substances against deterioration by oxidation which is catalyzed by the presence of or by contact with certain oxidation promoters. An important application of this invention resides in the reduction of the amount of gum formed in gasoline during storage due to the presence of small amounts of certain metals, their compounds or both. Another application is as a stabilizer for lubricating oils to retard discoloration, sludge formation, etc., due to catalytic oxidation.

It is the purpose of this invention to provide a class of deactivator compounds which reduce the catalytic effect of metal oxidation promoters, more particularly of iron, copper, chromium, cobalt, lead, and the compounds of copper, chromium, cobalt, and lead. It is another purpose to provide deactivators which when added to organic substances will remain active for a considerable length of time when subjected to oxidizing influences. Still another purpose is to render hydrocarbon oils insensitive to the catalytic oxidation of metals such as iron and copper for invariably during their useful life, the oils come in contact with one or the other of these metals.

Organic substances normally contact metals, or frequently contain small amounts of metals, usually dissolved in the form of a soluble salt, and it has been observed that the presence of such metals frequently has a detrimental effect on the stability of the substances. Inasmuch as bare traces of the metal may be very harmful and since removal of these last traces is extremely difficult, it is often not possible to eliminate this troublesome catalyst of the oxidation reaction.

It has already been suggested to reduce the susceptibility of organic substances to oxidation induced by the presence of copper, by adding to the organic substances certain deactivators which have the property of rendering the copper inactive. The deactivators heretofore suggested, comprise products of condensation of one mol of an aliphatic or aromatic primary diamine with two mols of salicylaldehyde or similar compounds. It is known from example, that the addition of these deactivators reduces the gum formation in the presence of dissolved copper as determined by the A. S. T. M. air jet method and also increases the induction period as tested by the Voorhees and Eisinger method described in S. A. E. J. 24, 584 (1929).

We have discovered the compounds, obtained by reacting one mol of an aromatic aldehyde having a hydroxyl radical in ortho position to the carbonyl radical with one mol of an aliphatic compound of not more than 12 carbon atoms which may be in a continuous or discon-

tinuous, straight or branched carbon chain, having one and preferably one only primary amine radical and preferably at least one hydroxyl radical, under conditions to eliminate water by the interaction of the carbonyl and primary amine radicals, possess the property of deactivating metallic copper, chromium, lead, cobalt, iron and the compounds of copper, chromium, lead and cobalt. Many of these compounds retain their activity after exposure to oxidizing influences. They have the general formula  $\text{o}-\text{HO}-\text{X}-\text{CH}=\text{N}-\text{Y}$  wherein X represents an aromatic nucleus, such as benzene, and Y represents an aliphatic radical having from 2 to 12 carbon atoms inclusive and containing a linkage between two carbon atoms of oxygen, sulfur or nitrogen other than the nitrogen and oxygen atoms to which said Y is attached.

The action of our deactivators appears to be specific for certain metals and their compounds. Different types of organic substances may be protected from the catalytic effect of metal oxidation promoters. The deactivators must be at least slightly soluble in the organic substance by itself or in the presence of a mutual solvent. Neutral and basic substances are in general more susceptible to the action of the deactivators than acids.

Aldehydes suitable to form deactivators with said aliphatic alcohols are, for example, salicylaldehyde, the homo-salicylaldehydes, trimethyl salicylaldehyde, isobutyl salicylaldehyde, ortho hydroxy naphthyl aldehyde, corresponding aldehydes of anthracene, etc. If desired, the aldehydes may contain substitution radicals, such as alkyl, halogen, amino, imino, hydrazine, ether, thioether, etc. radicals.

Aliphatic compounds of not more than 12 carbon atoms having one primary radical amine capable of forming deactivators with the salicylaldehydes mentioned previously are for example, the alkylamines of the general formula  $\text{NH}_2\text{R}$  wherein R is an aliphatic radical of 2 to 12 carbon atoms and which may contain the elements oxygen, sulfur and nitrogen, such as ethyl amine, butyl amine, isopropyl amine, amino ethyl methyl amine, amino propyl methyl amine, amino isopropyl methyl amine, n-heptyl amine, amino isoamyl propyl amine, beta amino ethyl ether, amino ethyl isopropyl ether, acetyl acetone amine, amino ethyl thiomethane, amino methyl thiohexane, amino ethyl thiopropane; or the hydroxy alkylamines of general formula



wherein R is an aliphatic radical of 2 to 12 carbon atoms and which may contain the elements oxygen, sulfur or nitrogen such as mono ethanolamine, mono butanolamine, mono dodecanol-amine, 1 amino 2 pentanol, 4 amino 2 pentanol,

hydroxy ethyl amino ethyl ether, hydroxy propyl amino ethyl ether, hydroxy propyl amino butyl ether, hydroxy propyl amino propyl ether, 1 hydroxy 2 methyl butyl amino propyl ether, the corresponding thio and imino ethers, sulfoxides and sulfones, such as hydroxy ethyl amino ethyl sulfoxides, hydroxy butyl amino ethyl sulfone, ketones and thioketones such as amino methyl isopropyl ketone, 1 hydroxy 5 amino pentanone 3, 1 hydroxy 5 amino pentathionone 3, hydroxy mono amino dipropyl acetone and acetals such as beta amino propionacetal and alpha amino butyric acetal acetone, etc. In addition suitable alcohols may contain other inorganic substituents particularly halogens.

Of the above, the hydroxy alkylamines are preferred yielding condensation products having the general formula  $\text{O}-\text{HO}-\text{X}-\text{CH}=\text{N}-\text{Y}-\text{OH}$  wherein X and Y have the same connotation as above. Particularly effective are those which in addition contain an ether, thioether or imino ether radical.

The reaction involved in producing our deactivators is well known and may be illustrated by the following equation:



The aliphatic chain of the amine should contain not more than 12 carbon atoms to produce relatively low molecular weight compounds, because the reaction between deactivator compounds and the metal is apparently one in which two molecules of deactivator are capable of capturing and deactivating not more than one atom of the metal. It is not therefore desirable to add too great an amount of dead load to the molecule of the deactivator.

The value of compounds as deactivators and suppressors of oxidation due to catalytic activity of the metals may be estimated by measuring the activities under at least two conditions, namely, before and after oxidation. Thus, for example, as applied to a gasoline, one may measure first, the extent to which it overcomes the adverse effect of the metal in lowering the induction period, second, the extent to which it reduces the initial copper dish gum value of the gasoline; and third, the extent to which it maintains low copper dish gum after accelerated oxidation.

To illustrate how the deactivators of this invention suppress the catalytic activity for example of copper, the deactivators were tested in gasoline containing 1 part per million of dissolved copper added as copper phenyl propionate. The results of the tests are shown in Table I.

Table I

| Deactivator added 2.5 mg./100 ml. gasoline                             | Induction period in hours |                                |
|------------------------------------------------------------------------|---------------------------|--------------------------------|
|                                                                        | When no added copper      | 1 P. P. M. of dissolved copper |
| None.....                                                              | 4.67                      | 1.88                           |
| Salicylal ethyl amine.....                                             | 4.83                      | 2.50                           |
| Salicylal ethanol amine.....                                           | 4.93                      | 2.25                           |
| Mono salicylal beta, beta' mono amino hydroxy diethyl imino ether..... | 5.25                      | 4.50                           |

In Table II below, the deactivation effects of mono salicylal beta beta' mono amino hydroxy diethyl imino ether on the copper dish gum and

induction periods before and after oxidation of a cracked gasoline are shown.

Table II

| Deactivator added 2.5 mg./100 ml. gasoline                             | Induction period, hours |                             | Copper dish gum, mg./100 ml. |                                    |
|------------------------------------------------------------------------|-------------------------|-----------------------------|------------------------------|------------------------------------|
|                                                                        | No added copper         | 1 P. P. M. dissolved copper | Initial                      | After 1 hour accelerated oxidation |
| None.....                                                              | 4.58                    | 1.67                        | 59.66                        | 128.17                             |
| Mono salicylal beta, beta' mono amino hydroxy diethyl imino ether..... | 5.17                    | 4.58                        | 11.13                        | 9.16                               |

It will be seen that the deactivator retained its ability to suppress the copper dish gum to the original low concentration even after exposure to oxidation conditions.

The effect of the deactivators in contact with lubricating oil is illustrated by the attached drawing representing a graph wherein is plotted the length of time in hours of oxidation against the amount of oxygen absorbed in the presence of metallic iron.

In this test, the oil is exposed to pure oxygen at atmospheric pressure and at a temperature of 150° C.

On the ordinate of the graph is plotted the mols of oxygen absorbed, on the abscissa is indicated the time of oxidation. Two curves are shown, curve 1 representing the rate of oxygen absorption in the absence of any deactivator and curve 2 representing the rate of oxygen absorption under identical conditions in the presence of 0.1% by weight of mono salicylal beta, beta' mono amino hydroxy diethyl imino ether.

It will be seen that the metallic iron was deactivated for a considerable length of time under the extremely severe conditions of the test.

Our deactivators also suppress the catalytic oxidation which may be caused by a combination of the various metal oxidation promoters. Thus for example, if gasoline containing dissolved copper is stored in an iron drum, our compounds deactivate both the dissolved copper and metallic iron.

Our products are active in various organic substances which are subject to deterioration by oxidation and which substances during their useful life come in contact with any of the metals or their compounds hereinbefore enumerated. Thus various refined and semi-refined hydrocarbon oils may be stabilized, such as gasoline, kerosene, special boiling point solvents, Diesel fuels, spray oils, lubricating oils, etc., pure hydrocarbons such as benzene, toluene, various liquid olefins, etc. Other substances capable of being protected are for example animal fats and oils, vegetable fats and oils, soaps, photographic developers, both natural and synthetic sulfonated and sulfated oils, essential oils, perfumes, cellulose acetate, rubber, various resins, etc.

The presence of antioxidants and other compounds in the substance to be desensitized, which compounds have the property of modifying the susceptibility of these substances toward non-catalytic oxidation such as ordinary oxidation inhibitors as used in gasoline, lubricating oil, rubber, fats, soaps, etc. may have an influence on the activity of deactivators, promoting or retarding their effectiveness.

The deactivators of this invention may be used in conjunction with other addition agents for

example, in gasoline, together with anti-knock compounds and anti-oxidants or in lubricating oils together with anti-oxidants, blooming agents, anti-corrosive, extreme pressure compounds, detergents, etc., or in Diesel fuels together with knock suppressors, anti-oxidants, etc. It is, however, desirable that the addition agent shall not raise the acidity of the substance to be desensitized to the point of greatly diminishing the activity of the deactivators.

The amounts of our deactivators to be added to the substances effectively to suppress the catalytic action of the metals or their compounds will naturally vary with the stability requirements of the treated product, as well as with the amount of metal contained in the organic substance if dissolved metal is the source of the instability.

In general quantities ranging from about .01% to 1% are useful and provide the necessary protection, although under certain circumstances, amounts outside of these limits may be used.

The metal deactivators may be added to the organic substances to be stabilized in any desired form. They may be added in solid or liquid form, mixed with other addition agents or dissolved in a solvent.

Some organic substances dissolve metals during their use. This, for instance, is the case with lubricating oils, electrical oils, gasolines, etc. When treating such substances with our compounds, it is often desirable to use an amount considerably in excess of that which is required to give it adequate initial protection. In such cases, the proper amounts of the deactivator may if desired be added during the use of the organic substances as may be required from time to time.

We claim as our invention:

1. An organic substance subject to deterioration through oxidation, which substance during its useful life comes in contact with an oxidation promoter selected from the group consisting of metallic iron, copper, chromium, lead, cobalt and the compounds of copper, chromium, lead and cobalt, containing a small amount of a deactivator having the general formula



wherein X represents an aromatic nucleus and Y represents an aliphatic radical having from 2 to 12 carbon atoms inclusive, and containing a linkage between two carbon atoms of an element selected from the group consisting of oxygen, sulfur and nitrogen other than the nitrogen and oxygen atoms to which said Y is attached.

2. An organic substance subject to deterioration through oxidation, which substance during its useful life comes in contact with an oxidation promoter selected from the group consisting of metallic iron, copper, chromium, lead, cobalt and the compounds of copper, chromium, lead and cobalt, containing a small amount of ortho salicylal beta beta' hydroxy amino di-ethyl imino ether.

3. The substance of claim 1 which contains from about 0.01% to about 1% by weight of the deactivator.

4. An organic substance subject to deterioration through oxidation, which substance during its useful life comes in contact with an oxidation promoter selected from the group consisting of metallic iron, copper, chromium, lead, cobalt and the compounds of copper, chromium, lead and cobalt, containing a small amount of a deactivator having the general formula



10 wherein X represents a mono-nuclear aromatic radical and Y represents an aliphatic radical having from 2 to 12 carbon atoms inclusive, and containing a linkage between two carbon atoms of an element selected from the group consisting of oxygen, sulfur and nitrogen other than the nitrogen and oxygen atoms to which said Y is attached.

5. A hydrocarbon fraction containing a small amount of a deactivator having the general formula



wherein X represents an aromatic nucleus and Y represents an aliphatic radical having from 2 to 12 carbon atoms inclusive, and containing a linkage between two carbon atoms of an element selected from the group consisting of oxygen, sulfur and nitrogen other than the nitrogen and oxygen atoms to which said Y is attached.

25 6. The method of increasing the stability of organic substances subject to deterioration through oxidation in contact with oxidation promoters selected from the group consisting of metallic iron, copper, chromium, lead, cobalt and the compounds of copper, chromium, lead and cobalt, which comprises incorporating in said organic substance a small amount of a metallic deactivator having the general formula



30 wherein X represents an aromatic nucleus and Y represents an aliphatic radical having from 2 to 12 carbon atoms inclusive, and containing a linkage between two carbon atoms of an element selected from the group consisting of oxygen, sulfur and nitrogen other than the nitrogen and oxygen atoms to which said Y is attached.

7. The method of prolonging the useful life of a hydrocarbon oil comprising incorporating therewith a small amount of a deactivator having the general formula



35 wherein X represents an aromatic nucleus and Y represents an aliphatic radical having from 2 to 12 carbon atoms inclusive, and containing a linkage between two carbon atoms of an element selected from the group consisting of oxygen, sulfur and nitrogen other than the nitrogen and oxygen atoms to which said Y is attached.

8. The method of prolonging the useful life of a hydrocarbon fraction which comprises adding thereto a small amount of ortho salicyl beta beta' hydroxy amino di-ethyl imino ether.

ELLIS R. WHITE.  
ERNEST L. WALTERS.